

## UNITED STATES PATENT OFFICE

1,925,526

## COLORING PAPER AND THE LIKE

Franz Dotzel, Ludwigshafen-on-the-Rhine, Germany, assignor to I. G. Farbenindustrie Aktiengesellschaft, Frankfort-on-the-Main, Germany

No Drawing. Application September 24, 1930,  
Serial No. 484,245, and in Germany October  
14, 1929.

## 12 Claims. (Cl. 8—5)

The present invention relates to coloring paper and the like.

It is already known that by coloring the substances serving for the preparation of paper, 5 pasteboard and the like or by coloring the paper itself with basic substantive and similar dyestuffs, mottled dyeings are often obtained. It is almost impossible to avoid this phenomenon even when all the precautions of the dyeing industry are taken, and it is due to the fact that the raw materials employed in the manufacture of paper have different affinities for the said dyestuffs. The phenomenon is therefore particularly marked with the use of paper from mixed 10 paper pulp. It has been tried to avoid this disagreeable effect by a treatment with tannin, but the results are not satisfactory.

I have now found that paper, which term is meant to include paper of any size, i. e. thin paper 20 as well as pasteboard and the like, can be colored in a manner free from the aforesaid objections with organic dyestuffs, such as basic, substantive and similar dyestuffs, and that therefore very valuable uniformly colored paper and 25 the like can be obtained by treating the substances serving for the preparation of the paper and the like during the working up thereof, or by treating the paper and the like themselves before, or at the same time as, coloring them, 30 with certain artificial tanning agents. After thorough mixing, the pulp is colored and sized in the usual manner. The artificial tanning agents suitable according to my present invention correspond to the general formula R-X-R in which 35 R defines a mono- or polycyclic aromatic nucleus, which may contain further non-aromatic substituents, and X is CH<sub>2</sub>, CH<sub>2</sub>-NH or S. Thus for example tanning compounds of the type



45 or



50 may be employed, the apparent polymeric nature of these compounds being defined by y which is higher than 1. These tanning materials may be prepared according to the U. S. Patents Nos.

55 1,191,480, 1,232,620, 1,237,405, 1,336,759, 1,421,722  
1,414,045, 1,254,364 and 1,203,069; the German

Patents Nos. 297,187, 297,188, 319,713 and 320,613 also describe the preparation of tanning materials suitable for carrying out the present invention. Particularly good results are obtained with 60 aromatic sulphonic acids corresponding to the last mentioned formula and their efficiency may be further increased by converting the acid tanning agents of the aforesaid nature into their alkali metal salts and adding, if desired, from 0.5 to 5 per cent their weight of alkali metal bisulphate.

The quantities of the artificial tanning agents employed are generally between 0.2 and 5 per cent of the paper pulp or paper, quantities between 0.5 and 1 per cent being usually satisfactory.

The good results obtainable according to the present invention are most surprising since tanning agents of unsymmetrical constitution, as for example phenyl methylene naphthyl compounds, do not prevent the disagreeable mottled 75 effects.

The following examples, in which coloring with dyestuffs particularly tending to give mottled dyeings is described, will further illustrate the nature of this invention, but the invention is not 80 restricted thereto.

## Example 1

From 0.5 to 1 per cent of the sodium salt of the synthetic tanning agent, prepared by condensation of  $\beta$ -naphthalene sulphonic acid and formaldehyde, and which has been dissolved in water, incorporated with from 1 to 3 per cent its weight of sodium bisulphite and rendered neutral, is added to the paper pulp in a hollander. 85 The pulp is then colored according to the desired shade, as for example with methylene Blue (Color Index, No. 922) or Cotton black RW extra (Color Index, No. 582) and sized in the usual manner. 90 In the product obtained all fibres are equally dyed.

## Example 2

1000 parts of a mixture of 7.5 parts of bleached sulphite pulp and 2.5 parts of unbleached sulphite pulp are worked in the paper machine together with 10 parts of the tanning agent, prepared by a condensation of phenol with sulphur and alkali, 500 parts of water and 5 parts of the dyestuff Vesuvine B (Color Index, No. 332). 105 Thoroughly uniform dyeings are obtained.

## Example 3

1000 parts of a mixture of equal parts of mechanical pulp and of unbleached sulphite pulp 110

are worked in the paper machine together with 10 parts of the tanning agent, prepared by a condensation of  $\beta$ -naphthalene sulphonic acid and formaldehyde, and which has been dissolved in 5 water and rendered neutral, 500 parts of water and 2 parts of Cotton black RW extra (Color Index, No. 582). The dyed paper or pasteboard does not show any mottled effects.

What I claim is:—

- 10 1. The process for coloring paper with an organic dyestuff selected from the class consisting of basic and substantive dyestuffs which comprises treating paper pulp at least during the dyeing operation with a synthetic tanning agent containing the grouping  $(R \cdot X \cdot R \cdot)^y$  in which  $y$  is greater than 1,  $R$  is an aromatic nucleus and  $X$  is  $CH_2$ ,  $CH_2-NH$  or  $S$ .
- 15 2. The process for coloring paper with an organic dyestuff selected from the class consisting of basic and substantive dyestuffs which comprises treating paper pulp at least during the dyeing operation with a synthetic tanning agent resulting from the condensation of a naphthalene sulphonic acid with formaldehyde.
- 20 3. The process for coloring paper with an organic dyestuff selected from the class consisting of basic and substantive dyestuffs which comprises treating paper pulp at least during the dyeing operation with a synthetic tanning agent resulting from the condensation of a naphthalene sulphonic acid with formaldehyde, and subsequent neutralization.
- 25 4. As a new article of manufacture paper comprising a synthetic tanning agent containing the grouping  $(R \cdot X \cdot R \cdot)^y$  in which  $y$  is greater than 1,  $R$  is an aromatic nucleus and  $X$  is  $CH_2$ ,  $CH_2-NH$  or  $S$ , which is uniformly colored by an organic dyestuff selected from the class consisting of basic and substantive dyestuffs.
- 30 5. As a new article of manufacture paper comprising a neutralized synthetic tanning agent containing the grouping  $(R \cdot X \cdot R \cdot)^y$  in which  $y$  is greater than 1,  $R$  is an aromatic nucleus and  $X$  is  $CH_2$ ,  $CH_2-NH$  or  $S$ , which is uniformly colored by an organic dyestuff selected from the class consisting of basic and substantive dyestuffs.
- 35 6. As a new article of manufacture paper comprising a synthetic tanning agent resulting from

the condensation of a naphthalene sulphonic acid and formaldehyde, which is uniformly colored by an organic dyestuff selected from the class consisting of basic and substantive dyestuffs.

7. As a new article of manufacture paper comprising a synthetic tanning agent resulting from the condensation of a naphthalene sulphonic acid and formaldehyde and subsequent neutralization with an alkali, which is uniformly colored by an organic dyestuff selected from the class consisting of basic and substantive dyestuffs. 80

8. As a new article of manufacture a preparation for uniformly coloring paper, comprising a neutralized synthetic tanning agent containing the grouping  $(R \cdot X \cdot R \cdot)^y$  in which  $y$  is greater than 1,  $R$  is an aromatic nucleus and  $X$  is  $CH_2$ ,  $CH_2-NH$  or  $S$  and a paper dyeing coloring material selected from the class consisting of basic and substantive dyestuffs. 90

9. As a new article of manufacture a preparation for uniformly coloring paper, comprising a synthetic tanning agent resulting from the condensation of a naphthalene sulphonic acid and formaldehyde and subsequent neutralization with an alkali and a paper dyeing coloring material selected from the class consisting of basic and substantive dyestuffs. 95

10. A composition of matter comprising paper pulp, a synthetic tanning agent containing the grouping  $(R \cdot X \cdot R \cdot)^y$  in which  $y$  is greater than 1,  $R$  is an aromatic nucleus and  $X$  is  $CH_2$ ,  $CH_2-NH$  or  $S$ , and an organic dyestuff selected from the class consisting of basic and substantive dyestuffs. 105

11. A composition of matter comprising paper pulp, a neutralized synthetic tanning agent resulting from the condensation of a naphthalene sulphonic acid and formaldehyde, and an organic dyestuff selected from the class consisting of basic and substantive dyestuffs. 110

12. A composition of matter comprising mechanical pulp and unbleached sulphite pulp, the sodium salt of a synthetic tanning agent resulting from the condensation of beta-naphthalene sulphonic acid and formaldehyde, and an organic dyestuff selected from the class consisting of basic and substantive dyestuffs. 120

FRANZ DOTZEL.

50

125

55

130

60

135

65

140

70

145

75

150